

**[54] PRESSURE-SENSITIVE RECORDING PAPER**

[75] Inventors: **Sadao Ishige; Takao Hayashi; Hiroharu Matsukawa**, all of Ashigara-Kamigun, Kanagawa, Japan

[73] Assignee: **Fuji Photo Film Co., Ltd., Kanagawa, Japan**

[22] Filed: **July 8, 1971**

[21] Appl. No.: **160,775**

**[30] Foreign Application Priority Data**

July 8, 1970 Japan..... 45/59698

[52] U.S. Cl..... **117/36.2, 117/36.8, 117/155 L, 260/38, 260/41.5 R**

[51] Int. Cl..... **B41m 5/22**

[58] Field of Search..... 117/36.2, 36.8, 36.9

**[56] References Cited****UNITED STATES PATENTS**

|           |        |                      |          |
|-----------|--------|----------------------|----------|
| 3,455,721 | 7/1969 | Phillips et al. .... | 117/36.2 |
| 3,509,174 | 4/1970 | Lin.....             | 117/36.2 |
| 3,592,677 | 7/1971 | Tsuboi et al. ....   | 117/36.2 |

Primary Examiner—Murray Katz

Attorney—Richard C. Sughrue et al.

**[57] ABSTRACT**

A pressure-sensitive recording paper comprising a layer of microcapsules containing a color former and a layer of a color developer, said layers coated on the same support or different supports, and at least one of said layers containing an ether derivative of an aromatic hydroxyl compound.

**6 Claims, 6 Drawing Figures**

FIG. 1



FIG. 2



FIG. 3



FIG. 4



FIG. 5



FIG. 6



## PRESSURE-SENSITIVE RECORDING PAPER

## BACKGROUND OF THE INVENTION

## 1. Field of the Invention

This invention relates to a pressure-sensitive recording paper, and more specifically, to a pressure-sensitive recording paper in which the coating layer contains an ether derivative of an aromatic hydroxyl compound.

## 2. Description of the Prior Art

Pressure-sensitive recording paper, as it has been known, for example, by U.S. Pat. Nos. 2,712,507, 2,730,465, and 2,730,457, is based on the utilization of microcapsules containing a solution of a substantially colorless organic compound (hereinafter, referred to "color former") and an electron-accepting adsorbent substance (hereinafter referred to "color developer").

In this application, an upper sheet means a support having coated thereon, a layer of microcapsules containing a color former; an intermediate sheet means a support having coated on one surface, a layer of microcapsules containing a color former and having coated on the opposite surface, a layer of color developer; and an undersheet means a support having coated thereon, a color developer. Further, a single-fold sheet means a support having coated thereon, a layer of microcapsules and a color developer, simultaneously.

Illustrative of the color formers are malachite green lactone, which is 3, 3-bis-(p-dimethylaminophenyl)-phthalide, benzoyl leuco methylene blue, crystal violet lactone, which is 3,3-bis(p-dimethylaminophenyl)-6-dimethylamino phthalide, Rhodamine B lactam, 3-dialkylamino-7-dialkylamino-fluorans, and 3-methyl-2,2'-spirobi(benzol[f]chromene).

On the other hand, the color developer, which is capable for forming a color dye when contacted with the color former, may be an active clay substance, such as acid clay, active clay, attapulgite, zeolite or bentonite, and organic acidic substances, such as succinic acid, tannic acid, gallic acid, pentachlorophenol and phenol resins.

The light resistance of the color dye formed by reaction of the color former and color developer depends upon the structure of the color former and also upon the color developer. The color developers now in wide use are clays, such as acidic clay. The light resistance of the color dye formed on an under sheet using this developer, although differing in the type of the color former, is generally poor except benzoyl leuco methylene blue. Hence, when such a paper is left indoors or exposed to sunlight, the density of the color dye formed on the paper is easily reduced; that is, the color changes easily. Accordingly, the commercial availability of pressure-sensitive recording paper is reduced.

The color former most often employed is a mixture of crystal violet lactone and benzoyl leuco methylene blue. Since crystal violet lactone has a very poor resistance to light, the color dye formed on the color developer sheet fades when allowed to stand indoors or exposed to sunlight. Consequently, only the light blue color formed from methylene blue remains, which obviously reduces the commercial value of the recording paper. For the production of a black color or green color, 3-dibenzylamino-7-diethylaminofluorane is used. It develops a green color on acid clay, but changes to red brown on standing indoors or on exposure to sunlight. Accordingly, the black or green color formed by 3-benzylamino-7-diethylaminofluorane assumes a red-

dish color on standing indoors or exposure to sunlight, resulting in a reduction in the commercial value of the pressure-sensitive recording paper.

## SUMMARY OF THE PRESENT INVENTION

It is an object of this invention to provide a pressure-sensitive recording paper having excellent resistance to light.

The foregoing object is achieved by incorporating at least one ether derivative of an aromatic hydroxyl compound in the coating layer of the pressure-sensitive recording paper.

## DETAILED DESCRIPTION OF THE INVENTION

Examples of the ether derivative of the aromatic hydroxyl compound applicable to this invention include p-chloroanisole, p-methylanisole, p-acetoxyanisole, p-acetaminoanisole, o-chloroanisole, m-chloroanisole, N-β-cyanoethyl —p-anisidine, p-methoxyacetophenone, p-methoxybenzophenone, 2,2-bi(p-methoxyphenyl)propane, catechol dimethyl ether, resorcinol dimethyl ether, hydroquinone dimethyl ether, catechol diethyl ether, resorcinol dipropyl ether, hydroquinone dibutyl ether, p-methoxybenzoic acid ethyl ester, p-ethoxybenzenesulfonamide, 1-phenoxy-2-cyanoethane, 1-phenoxy-2-hydroxyethane, 1-phenoxy-2-chloroethane, diphenyl ether, hydroquinone dibenzyl ether, 1,2-dimethoxy-4-(p-methoxyphenoxy)benzene, 1,4-dimethoxy-2-octadecyl benzene, 1-(p-<sup>a</sup>,<sup>a</sup>-dimethyl-benzylphenoxy)-4-ethoxybenzene, 1-ethoxy-2,3-methylene dioxy benzene, 2,5-dimethoxybenzenesulfonamide, 1,4-dibutyl-2,5-dimethoxybenzene, 1,4-diethoxyanthracene, 5-methyl-1,4-diethoxyanthracene, 8-chloro-1,4-diethoxyanthracene, 9,10-dimethoxyanthracene, 4-methyl-9,10-dimethoxy-anthracene, 7-chloro-9,10-dimethoxyanthracene, 1-methoxyanphthalene, 2-ethoxynaphthalene, 4-chloro-1-methoxynaphthalene, 5-methyl-1-methoxynaphthalene 8-chloro-2-ethoxynaphthalene, and 6-propyl-2-ethoxynaphthalene.

These ether derivatives of aromatic hydroxyl compounds may be microencapsulated. In this case, the compounds may be microencapsulated with at least one color former. It is also possible to add these compounds to a color developer.

The acceptable amount of the ether derivative of the aromatic hydroxyl compound applicable to this invention ranges from 10 to 200% by weight based on the weight of the color former used, or 0.2 to 10% based on the weight of the color developer used.

Microcapsules containing the color former may be produced, for example, by the process disclosed in U.S. Pat. No. 2,700,458, but the process of microcapsulation is not limited to such, since the present invention is directed to incorporation of the ether derivative.

A better understanding of the present invention will be attained from the following examples, which are merely intended to be illustrative and not limitative of the present invention. All parts are by weight unless otherwise stated.

## Example 1

10 parts of acid-treated pig skin gelatin and 10 parts of gum arabic were dissolved in 400 parts of water at 40° C. As an emulsifier, 0.2 part of Turkey red oil was added. To this solution was added 40 parts of a color

former oil in which 3% of hydroquinone dimethyl ether had been dissolved. This mixed solution was emulsified and dispersed. The color former oil consisted of a solution of four parts of diphenyl chloride and one part of kerosene in which 2% of crystal violet lactone was dissolved.

When the average sizes of the oil droplets reached 5 microns, the emulsification was stopped. Water at 40° C. was added to the emulsion to make 900 parts, and stirring was continued. In this case, caution should be taken not to lower the temperature below 40° C. Thereafter, 10% acetic acid was added to adjust the pH of the liquid to 4.0 and thereby induce coacervation. Stirring was further continued for 20 minutes, and then the mixture was cooled with ice water to cause gelation of coacervate films deposited around the oil droplets. When the temperature of the liquid became 20° C., seven parts of a 37% formaldehyde solution were added. When the temperature dropped to 10° C., an aqueous 15% solution of sodium hydroxide was added to adjust the pH to 9. The addition of the sodium hydroxide was performed with meticulous care so as not to coagulate the system. With continued stirring, the liquid was heated to 50° C. After cooling to 30° C., the microcapsule liquid thus obtained was coated onto a paper having a unit weight of 40 g/m<sup>2</sup> in an amount of 6 g/m<sup>2</sup> as solid content, and dried to make an upper sheet of pressure sensitive recording paper.

#### Example 2

To 40 parts of a color former oil consisting of a solution of 2% crystal violet lactone in an oil composed of four parts of diphenyl chloride and one part of kerosene was dissolved 3%, based on the color former oil, of N-( $\beta$ -cyanoethyl) p-anisidine. The solution was microencapsulated in the same manner as in Example 1. The resulting microcapsule liquid was coated onto a paper having a unit weight of 40 g/m<sup>2</sup> in an amount of 6 g/m<sup>2</sup> as solid content, and dried to form an upper sheet of pressure-sensitive recording paper.

#### Example 3

To 40 parts of a color former oil obtained by dissolving 2% crystal violet lactone in an oil consisting of four parts of diphenyl chloride and one part of kerosene was dissolved 3% by weight, based on the oil, of p-methylanisole. The solution was microencapsulated in the same way as in Example 1. The resulting microcapsule liquid was coated onto a paper having a unit weight of 40 g/m<sup>2</sup> in an amount of 6 g/m<sup>2</sup> as solid content, and dried to form an upper sheet of pressure-sensitive recording paper.

#### COMPARATIVE EXAMPLE 1

40 parts of a color former oil obtained by dissolving 2% crystal violet lactone in an oil consisting of four parts of diphenyl chloride and one part of kerosene was microencapsulated in the same manner as in Example 1. The resulting microcapsule liquid was coated onto a paper having a unit weight of 40 g/m<sup>2</sup> in an amount of 6 g/m<sup>2</sup> as solid content, and dried to form an upper sheet of pressure-sensitive recording paper.

In order to perform comparative tests on the upper sheets obtained in Examples 1 to 3 and Comparative Example 1, an under sheet was produced as follows:

Method of production of under sheet.

Eight parts of a 20% sodium hydroxide was added to 300 parts of water, and with stirring, 100 parts of acid clay (product of the Mizusawa Kagaku Kogyo Kabushiki Kaisha) was gradually added. After thorough stirring, the stirring was made slower, and 20 parts (as solid content) of styrene butadiene rubber latex ("Dow 620", tradename manufactured by the Dow Chemical Company) was gradually added to form a coating solution. The coating solution was coated on raw paper having a unit weight of 40 g/m<sup>2</sup> in an amount of 10 g/m<sup>2</sup> as solid content, and dried to form an under sheet of pressure sensitive recording paper for test purposes.

#### Comparative test 1

Each of the upper sheets of Examples 1, 2, and 3 and Comparative Example 1 was superposed on the under sheet, and a pressure of 600 Kg/cm<sup>2</sup> was applied to produce a color. After allowing the specimen to stand for 1 hour in dark, the spectral absorption curve (fresh) in a wave-length region of 700 to 380 m $\mu$  was measured with respect to the developed color. The results are shown in FIG. 1, (1) to (4).

The measurement of the spectral absorption curve was performed using a Beckman spectrophotometer, Type DB. The light resistance values were obtained as follows:

$$\text{Light resistance} = \frac{\text{density at the absorption maximum after sunlight exposure}}{\text{fresh density at the absorption maximum}} \times 100$$

The results obtained are shown in Table 1 below:

TABLE 1.—LIGHT RESISTANCE VALUES OF CRYSTAL VIOLET LACTONE AT THE ABSORPTION MAXIMUM AFTER SUNLIGHT EXPOSURE

|                             | One hour sunlight exposure (percent) | Three hour sunlight exposure (percent) | Numbers of Figure 1 |
|-----------------------------|--------------------------------------|----------------------------------------|---------------------|
| Example 1.....              | 65.1                                 | 41.3                                   | (1)                 |
| Example 2.....              | 59.1                                 | 32.6                                   | (2)                 |
| Example 3.....              | 54.2                                 | 32.1                                   | (3)                 |
| Comparative Example 1 ..... | 46.4                                 | 21.6                                   | (4)                 |

In FIG. 1, the fresh density is represented by A, the density after 1 hour exposure to sunlight is represented by B, and the density after 3 hours exposure to sunlight is represented by C (the same will apply to FIGS. 2 to 6).

The foregoing results demonstrate that the use of the ether derivative of the aromatic hydroxyl compound leads to an increase in the light resistance of crystal violet lactone.

#### Example 4

55 To 40 parts of a color former oil obtained by dissolving 2% 3-methyl-2,2'-spirobi(benzo[f]chromene) in an oil consisting of four parts of diphenyl chloride and one part of kerosene was dissolved 3%, based on the oil, of hydroquinone dimethyl ether. The solution was microencapsulated in the same way as set forth in Example 1. The resulting microcapsule solution was coated on a paper having a unit weight of 40 g/m<sup>2</sup> in an amount of 6 g/m<sup>2</sup> as solid content, and dried to form an upper sheet of pressure-sensitive recording paper.

#### Example 5

In 40 parts of a color former oil obtained by dissolving 2% 3-methyl-2,2'-spirobi(benzo[f]chromene) in an

oil consisting of four parts of diphenyl chloride and one part of kerosene was dissolved 3%, based on the oil, of *N*-( $\beta$ -cyano-ethyl)-*p*-anisidine. The solution was microencapsulated in the same way as in Example 1. The resulting microcapsule liquid was coated on a paper having a unit weight of 40 g/m<sup>2</sup> in an amount of 6 g/m<sup>2</sup> as solid content, and dried to form an upper sheet of pressure-sensitive recording paper.

Example 6

In 40 parts of a color former oil obtained by dissolving 2% 3-methyl-2,2'-spirobi(benzo[f]chromene) in an oil consisting of four parts of diphenyl chloride and one part of kerosene was dissolved 3%, based on the oil, of *p*-methylanisole. The solution was microencapsulated in the same way as set forth in Example 1. The resulting microcapsule liquid was coated on a paper having a unit weight of 40 g/m<sup>2</sup> in an amount of 6 g/m<sup>2</sup> as solid content, and dried to form an upper sheet of pressure-sensitive recording paper.

COMPARATIVE EXAMPLE 2

40 parts of a color former oil obtained by dissolving 2% 3-methyl-2,2'-spirobi(benzo[f]chromene) in an oil consisting of four parts of diphenyl chloride and one part of kerosene was microencapsulated in the same way as in Example 1. The resulting microcapsule solution was coated on a paper having a unit weight of 40 g/m<sup>2</sup> in an amount of 6 g/m<sup>2</sup> as solid content, and dried to form an upper sheet of pressure-sensitive recording paper.

Comparative test 2

Each of the upper sheets obtained in Examples 4, 5 and 6 and Comparative Example 2 was superposed on the test under sheet, and a pressure of 600 Kg/cm<sup>2</sup> was applied to develop a color. After allowing the paper to stand for one hour in dark, the spectral absorption curve (fresh) of the developed color in a wavelength region of 700 to 380m $\mu$  was measured. The measurement was also made after exposing the specimens to sunlight for 1 hour and 3 hours, respectively. The results are shown in FIG. 2, (1) to (4). The light resistance values were calculated in the same way as in Comparative Test 1. The results are shown in Table 2:

TABLE 2.—LIGHT RESISTANCE VALUES OF 3-METHYL-2,2'-SPIROBI(BENZO[F]CHROMENE) AT THE ABSORPTION MAXIMUM AFTER SUNLIGHT EXPOSURE

|                            | One hour sunlight exposure (percent) | Three hour sunlight exposure (percent) | Numbers of Figure 2 |
|----------------------------|--------------------------------------|----------------------------------------|---------------------|
| Example 4.....             | 87.6                                 | 83.8                                   | (1)                 |
| Example 5.....             | 86.5                                 | 84.7                                   | (2)                 |
| Example 6.....             | 78.6                                 | 75.4                                   | (3)                 |
| Comparative Example 2..... | 73.5                                 | 67.2                                   | (4)                 |

It is seen from the foregoing results that the light resistance of 3-methyl-2,2'-spirobi(benzo[f]chromene) is increased by using the ether derivative of the aromatic hydroxyl compound, and its color changes very little.

Example 7

To 40 parts of a color former oil obtained by dissolving 5% 3-dibenzylamino-7-diethylaminofluoran in an oil consisting of four parts of diphenyl chloride and one part of kerosene was dissolved 3%, based on the oil, of hydroquinone dimethyl ether. The solution was micro-

encapsulated in the same way as set forth in Example 1. The resulting microcapsule liquid was coated on a paper having unit weight of 40g/m<sup>2</sup> in an amount of 6 g/m<sup>2</sup> as solid content, and dried to form an upper sheet of pressure-sensitive recording paper.

Example 8

To 40 parts of a color former oil obtained by dissolving 5% 3-dibenzylamino-7-diethylaminofluoran in an oil consisting of four parts of diphenyl chloride and one part of kerosene was dissolved 3%, based on the oil, of *N*-( $\beta$ -cyanoethyl)-*p*-anisidine. The solution was microencapsulated in the same way as in Example 1. The resulting microcapsule liquid was coated on raw paper having a unit weight of 40 g/m<sup>2</sup> in an amount of 6 g/m<sup>2</sup> as solid content, and dried to form an upper sheet of pressure-sensitive recording papers.

Example 9

To 40 parts of a color former oil obtained by dissolving 5% 3-dibenzylamino-7-diethylaminofluoran in an oil consisting of four parts of diphenyl chloride and one part of kerosene was dissolved 3%, based on the oil, of *p*-methylanisole. The solution was microencapsulated in the same way as set forth in Example 1. The resulting microcapsule liquid was coated on a paper having a unit weight of 40 g/m<sup>2</sup> in an amount of 6 g/m<sup>2</sup> as solid content, and dried to form an upper sheet of pressure-sensitive recording paper.

COMPARATIVE EXAMPLE 3

40 parts of a color former oil obtained by dissolving 5% 3-dibenzylamino-7-diethylaminofluoran in an oil consisting of four parts of diphenyl chloride and one part of kerosene was microencapsulated in the same way as in Example 1. The resulting microcapsule liquid was coated on a paper having a unit weight of 40 g/m<sup>2</sup> in an amount of 6 g/m<sup>2</sup> as solid content, and dried to form an upper sheet of pressure-sensitive recording paper.

Comparative test 3

Each of the upper sheets obtained in Examples 7, 8 and 9 and Comparative Example 3 was superposed on the test under sheet, and a pressure of 600 Kg/cm<sup>2</sup> was applied to develop a color. After allowing the paper to stand for one hour in dark, the spectral absorption curve (fresh) of the developed color in a wavelength region of 700 to 380 m $\mu$  was measured. The spectral absorption curve of the color after exposure to sunlight for 1 hour and 3 hours, respectively, was also measured. The results are shown in FIG. 3, (1) to (4). The light resistance values were calculated in the same way as shown in Comparative Test 1. The results are shown in Table 3.

TABLE 3.—LIGHT RESISTANCE VALUE OF 3-BENZYLAMINO-7-DIETHYLAMINOFUORAN AT THE ABSORPTION MAXIMUM AFTER SUNLIGHT EXPOSURE

|                            | One hour sunlight exposure (percent) | Three hour sunlight exposure (percent) | Numbers of Figure 3 |
|----------------------------|--------------------------------------|----------------------------------------|---------------------|
| Example 7.....             | 84.8                                 | 75.8                                   | (1)                 |
| Example 8.....             | 84.1                                 | 76.1                                   | (2)                 |
| Example 9.....             | 83.5                                 | 72.6                                   | (3)                 |
| Comparative Example 3..... | 69.1                                 | 59.9                                   | (4)                 |

The foregoing results show that the light resistance of 3-dibenzyl-amino-7-diethylaminofluoran is also in-

creased by using the ether derivative of the aromatic hydroxyl compound.

On the basis of the spectral absorption curves in FIG. 3, (1) to (4), the movement of the absorption maximum ( $\lambda_1$ ) by sunlight exposure is tabulated in Table 4 below:

TABLE 4.—MOVEMENT OF THE ABSORPTION MAXIMUM  $\lambda_1$  OF 3-DIBENZYLAMINO-7-DIETHYLAMINOFLUORAN BY SUNLIGHT EXPOSURE FOR THE SPECIFIED TIME

|                            | Fresh $\lambda_1$<br>(m $\mu$ ) | $\lambda_1$ after<br>one hour<br>sunlight<br>exposure<br>(m $\mu$ ) | $\lambda_1$ after<br>three hour<br>sunlight<br>exposure<br>(m $\mu$ ) |
|----------------------------|---------------------------------|---------------------------------------------------------------------|-----------------------------------------------------------------------|
| Example 7.....             | 600                             | 580                                                                 | 560                                                                   |
| Example 8.....             | 600                             | 580                                                                 | 550                                                                   |
| Example 9.....             | 600                             | 585                                                                 | 550                                                                   |
| Comparative Example 3..... | 600                             | 545                                                                 | 485                                                                   |

As is seen from these results, the movement of the absorption maximum of 3-dibenzylamino-7-diethylamino-fluoran by sunlight exposure was reduced by using the ether derivative of the aromatic hydroxyl compound. This means that there was little change in color.

Compared with other color formers, the ether derivatives of the aromatic hydroxyl compounds exhibited the effect of increasing the light resistance of the color formers and preventing their discoloration.

#### Example 10

Eight parts of a 20% sodium hydroxide solution (as a dispersant) was added to 300 parts of dispersing water, and with stirring, 100 parts of acid clay (Mixusawa Kagaku Kogyo Kabushiki Kaisha) was added gradually. With stirring, a solution of 2 g of hydroquinone dimethyl ether in 30 cc of methanol was gradually added. The stirring was then made slower, and 20 parts (solid content) of styrene butadiene rubber latex (Dow 620; tradename, manufactured by the Dow Chemical Company) was gradually added to form a coating solution. The coating solution was coated on a paper having a unit weight of 40g/m<sup>2</sup> in an amount of 10g/m<sup>2</sup> as solid content, and dried to form an under sheet of pressure-sensitive recording paper.

#### COMPARATIVE EXAMPLE 4

Same as the test under sheets as used in Examples 1 to 9 and Comparative Examples 1 to 3.

Upper leaf sheets for test purposes

For comparative tests on the under sheets, the upper sheets of Comparative Examples 1, 2 and 3 were used.

#### Comparative test 4

The upper sheet of Comparative Example 1 was superposed on each of the under sheets obtained in Example 10 and Comparative Example 4, and a pressure of 600 Kg/cm<sup>2</sup> was applied to develop a color. After allowing the paper to stand for 1 hour in dark, the spectral absorption curve (fresh) in a wavelength region of 700 to 380 m $\mu$  was measured. The spectral absorption curve of the developed color after sunlight exposure for 1 hour and 3 hours, respectively, was also measured. The results are shown in FIG. 4, (1). The result of Comparative Example 4 was the same as that of Comparative Example 1. The light resistance values were calculated in the same way as in Comparative Test 1. The results are given in Table 5:

TABLE 5.—LIGHT RESISTANCE VALUE OF CRYSTAL VIOLET LACTONE AT THE ABSORPTION MAXIMUM AFTER SUNLIGHT EXPOSURE

|                            | One hour<br>sunlight<br>exposure<br>(percent) | Three hour<br>sunlight<br>exposure<br>(percent) | Figures      |
|----------------------------|-----------------------------------------------|-------------------------------------------------|--------------|
| Example 10.....            | 55.0                                          | 32.1                                            | Figure 4 (1) |
| Comparative Example 4..... | 46.4                                          | 21.6                                            | Figure 1 (2) |

10 The foregoing results indicate that hydroquinone dimethyl ether, in the presence of the color developer, improved the light resistance of crystal violet lactone. Comparative test 5

15 The upper sheet [containing microcapsules of 3-methyl-2,2'-spirobi(benzo[f]chromene)] was superposed on each of the under sheets obtained in Example 10 and Comparative Example 4, and a pressure of 600 Kg/cm<sup>2</sup> was applied to develop a color. After allowing the paper to stand for 1 hour in a dark place, the spectral absorption curve (fresh) in a wavelength region of 700 to 380 m $\mu$  was measured. The spectral absorption curve of the developed color after sunlight exposure for 1 hour and 3 hours, respectively, was also measured.

20 The results are shown in FIG. 5 (1). The light resistance values were calculated in the same way as in Comparative Test 1. The results are given in Table 6. The result of Comparative Example 4 was the same as that of Comparative Example 2.

30 TABLE 6.—LIGHT RESISTANCE VALUE OF 3-METHYL-2,2'-SPIROBI(BENZO[F]CHROMENE) AT THE ABSORPTION MAXIMUM AFTER SUNLIGHT EXPOSURE

|                            | One hour<br>sunlight<br>exposure<br>(percent) | Three hour<br>sunlight<br>exposure<br>(percent) | Numbers of<br>Figures |
|----------------------------|-----------------------------------------------|-------------------------------------------------|-----------------------|
| Example 10.....            | 92.9                                          | 87.4                                            | Figure 5 (1)          |
| Comparative Example 4..... | 73.5                                          | 67.2                                            | Figure 2 (4)          |

35 The foregoing results illustrate that hydroquinone dimethyl ether, in the presence of the color developer, improved the light resistance of 3-methyl-2,2'-spirobi(benzo[f]chromene) and prevented its discoloration. Comparative test 6

40 The upper sheet of Comparative Example 3 (containing microcapsules of 3-benzylamino-7-diethylamino-fluoran) was superposed on each of the under sheets obtained in Example 10 and Comparative Example 4, and a pressure of 600 Kg/cm<sup>2</sup> was applied to develop a color. After allowing the paper to stand for 1 hour in dark, the spectral absorption curve (fresh) in a wavelength region of 700 to 380 m $\mu$  was measured. The spectral absorption curve of the developed color after sunlight exposure for 1 hour and 3 hours, respectively, was also measured.

45 The results are shown in FIG. 6, (1) to (2). The result of Comparative Example 4 was the same as that of Comparative Example 3. The light resistance values were calculated in the same way as in Comparative Test 1. The results are given in Table 7:

50 TABLE 7.—LIGHT RESISTANCE VALUE OF 3-DIBENZYLAMINO-7-DIETHYLAMINOFLUORAN AT THE ABSORPTION MAXIMUM AFTER SUNLIGHT EXPOSURE

|                            | One hour<br>sunlight<br>exposure<br>(percent) | Three hour<br>sunlight<br>exposure<br>(percent) | Numbers of<br>Figures |
|----------------------------|-----------------------------------------------|-------------------------------------------------|-----------------------|
| Example 10.....            | 80.2                                          | 71.4                                            | Figure 6 (1)          |
| Comparative Example 4..... | 69.1                                          | 59.9                                            | Figure 3 (4)          |

The movement of the absorption maximum  $\lambda_1$  by sunlight exposure, based on FIG. 6,(1) to (2), is shown in Table 8:

TABLE 8.—MOVEMENT OF THE ABSORPTION MAXIMUM  $\lambda_1$  OF 3-DIBENZYLAMINO-7-DIETHYLAMINOFLUORAN BY SUNLIGHT EXPOSURE

|                            | Fresh $\lambda_1$<br>(m $\mu$ ) | $\lambda_1$ after<br>one hour<br>sunlight<br>exposure<br>(m $\mu$ ) | $\lambda_1$ after<br>three hour<br>sunlight<br>exposure<br>(m $\mu$ ) |
|----------------------------|---------------------------------|---------------------------------------------------------------------|-----------------------------------------------------------------------|
| Example 10.....            | 600                             | 580                                                                 | 550                                                                   |
| Comparative Example 4..... | 600                             | 545                                                                 | 485                                                                   |

The above results show that hydroquinone dimethyl ether increases the light resistance of 3-dibenzylamino-7-diethylaminofluoran and markedly prevents its discoloration.

With other ether derivatives of aromatic hydroxyl compounds, the same results as those obtained in Comparative Tests 1 to 6 were obtained.

Although the present invention has been adequately described in the foregoing specification and examples included therein, it is readily apparent that various changes and modifications may be made without departing from the scope and spirit thereof.

What is claimed is:

1. In a pressure-sensitive recording paper, comprising a layer of microcapsules containing a substantially colorless organic compound color former and a layer of a color developer selected from the group consisting of an acid clay substance, an organic acidic substance, and a phenol resin, which color former and color developer react upon contact to yield a distinguishable color dye reaction product, said layers being coated on the same support or different supports, the improvement: 35

wherein at least one of said layers contains an ether derivative of an aromatic hydroxyl compound which increases the resistance of said color dye reaction product to fading upon exposure to light, the amount of said ether derivative ranging from 10 to 400% by weight based on the weight of the color former or from 0.2 to 10% by weight based on the weight of the color developer.

2. The pressure-sensitive recording paper of claim 1, wherein said ether derivative is a member selected 45

from the group consisting of p-chloroanisole, p-methylanisole, p-acetoxyanisole, p-acetaminoanisole, o-chloroanisole, m-chloroanisole, N- $\beta$ -cyanoethyl-p-anisidene, p-methoxyacetophenone, p-methoxybenzophenone, 2,2-bi(p-methoxyphenyl) propane, catechol dimethyl ether, resorcinol dimethyl ether, hydroquinone dimethyl ether, catechol diethyl ether, resorcinol dipropyl ether, hydroquinone dibutyl ether, p-methoxybenzoic acid ethyl ester, p-ethoxybenzenesulfonamide, 1-phenoxy-2-cyanoethane, 1-phenoxy-2-hydroxyethane, 1-phenoxy-2-chloroethane, diphenyl ether, hydroquinone dibenzyl ether, 1,2-dimethoxy-4-(p-methoxyphenoxy) benzene, 1,4-dimethoxy-2-octadecyl benzene, 1-(p- $\alpha$ , $\alpha$ -dimethylbenzylphenoxy)-4-ethoxybenzene, 1-ethoxy-2,3-methylene dioxy benzene, 2,5-dimethoxybenzenesulfonamide, 1,4-dibutyl-2, 5-dimethoxybenzene, 1,4-diethoxyanthracene, 5-methyl-1,4-diethoxyanthracene, 8-chloro-1,4-diethoxyanthracene, 9,10-dimethoxyanthracene, 4-methyl-9,10-dimethoxyanthracene, 7-chloro-9,10-dimethoxyanthracene, 1-methoxynaphthalene, 2-ethoxynaphthalene, 4-chloro-1-methoxynaphthalene, 5-methyl-1-methoxynaphthalene, 8-chloro-2-ethoxynaphthalene, and 6-propyl-2-ethoxynaphthalene.

3. The pressure-sensitive recording paper of claim 1, wherein said color former is a member selected from the group consisting of malachite green, benzoyl leuco methylene blue, crystal violet lactone, Rhodamine B lactam, 3-dialkylamino-7-dialkylamino-fluorans, and 3-methyl-2,2'-spirobi(benzo[f]chromene).

4. The pressure-sensitive recording paper of claim 1, wherein said color developer is a member selected from the group consisting of active clay substances and organic acidic substances.

5. The pressure-sensitive recording paper of claim 4, wherein said active clay substance is a member selected from the group consisting of active clay attapulgite, zeolite and bentonite.

6. The pressure-sensitive recording paper of claim 4, wherein said organic acidic substance is a member selected from the group consisting of succinic acid, tannic acid, gallic acid, pentachlorophenol, and phenol resins.

\* \* \* \* \*